

## UNITED STATES PATENT OFFICE

WALTER BROADBRIDGE, EDWIN EDSER, AND WILLIAM WARWICK STENNING, OF LONDON, ENGLAND, ASSIGNEES TO MINERALS SEPARATION NORTH AMERICAN CORPORATION, OF NEW YORK, N. Y., A CORPORATION

## PRODUCTION OF COKE

No Drawing. Original application filed November 20, 1922, Serial No. 602,251, and in Great Britain November 29, 1921. Divided and this application filed April 22, 1926. Serial No. 103,968.

This invention relates to the production of coke from coal, and is herein described as applied to the production of coke of relatively much lower ash than the lump raw coal used 5 as raw material.

In our previous United States Patent No. 1,504,861 we have described various processes of producing agglomerates from impure coal, coal dumps and the like adapted for the making 10 of briquettes. We have now found that particles of coal and the like can be flocculated under such conditions as to facilitate the separation of water therefrom without the production of briquettes under water-expelling 15 pressure.

We have found that various agents such as certain oils, tars and other hydrocarbons or carbonaceous liquids which are incapable of forming briquettes of the carbonized materials such as coal under the conditions hereinafter described have the properties—

- (1) Of coating the coal particles, and
- (2) Of causing the coal particles, when so coated, to flocculate together.

We have further found that this flocculating effect occurs with very small quantities of the agents referred to when the coal particles are agitated with the flocculating agent in sufficient water to make a mobile pulp, 20 preferably with aeration. The quantities of the reagents may be very small, (from 3 to 10% of the weight of the coal, for example) sufficient only to coat the coal particles with a thin film of the agent like a varnish, and

30 quite insufficient to fill the interstitial spaces between the flocculated particles. The flocculates include in the interstitial spaces a large proportion of water, but owing to the fact that the surfaces of the particles have 40 become repellent of the water, it is possible to remove contained water by filtration or draining, preferably assisted by pressure, and thus the drying of the particles becomes a simple matter.

45 The removal of the water associated with the coated and flocculated particles may be assisted by pressure, but it is to be understood that it is not an object of the present invention to convert the materials into briquettes, 50 and the coating and flocculating agent does

not perform the function of a binding medium to form briquettes.

The presence of the flocculating agent assists the coking of special types of coal which would otherwise be unsuitable for making 55 coke. According to the present invention therefore a process for producing coke may consist in agitating a pulp of suitably powdered coal with a suitable flocculating agent under such conditions that the coal is flocculated and coated with a water-repellant coating adapted to be partly volatilized in a subsequent coking operation and having so little adhesiveness as not to cause the coal to form into hard briquettes under water-expelling 60 pressure, separating and draining the flocculated coal, and coking the drained coal.

The tarry residue from the volatilized matter, or some part of this, may be utilized as the flocculating agent in treating further masses 70 of carbonaceous material.

The quantity of the flocculating agent employed should be sufficient to produce the flocculation at the temperature of the circuit water. It may be reduced by using a heated 75 circuit, but preferably the treatment is carried out at atmospheric temperature. From 3 to 5% has been found sufficient when using as agent a product such as anthracene oil, and coal-tar, coal-tar oil and other reagents may 80 be employed in like proportion.

The following examples illustrate various procedures in accordance with the invention:—

## Example I

Coal from a Durham Colliery was ground to pass a screen of 0.4 mm. aperture. The ground coal was concentrated by flotation, using 0.23 kilos cresol and 0.06 kilos kerosene 90 oil per ton of coal. The concentrates removed had a water-solid ratio of 1.3 : 1.

The concentrates with their associated water were placed in a vessel of square horizontal section and were agitated by an impeller rotating with a peripheral velocity of about 200 meters per minute. By-product coke-oven coal-tar was added during the agitation, the quantity of tar amounting to 4% 95 of the weight of the dry concentrates. The 100

test was carried out at room temperature. The coal became intensely flocculated and readily separable from the water. Removal of the bulk of the water was effected by draining; it could be assisted if desired by subjecting the flocculated coal to compression. Under a pressure of 310 kilos per square cm. the coal became substantially free from water, so much so that on drying it in a water oven at a temperature of 100° C. for a period of 3½ hours, the weight diminished by 2.7%, which indicates the reduction in water content.

The coal was thus formed into a cake which, however, could be easily crumbled between the fingers. It will be understood that it is not essential to compress the coal into cakes in this way although this may be done both to assist removal of the water and to facilitate handling of the treated material.

A full oven charge (about 7 tons) of the above coal, flocculated as described above and pressed into soft ovoids at a pressure of about 310 kilos per sq. cm., was coked, the time of heating being about 30 hours. The resulting coke was of excellent quality, specially suitable for metallurgical use; it showed no trace of ovoid structure, and sustained a pressure of 160 kilograms per sq. cm. without crushing.

It was found that the oven capacity was increased by more than 12%.

#### Example II

Coal from Powell Duffryn Collieries was ground to pass a screen with an aperture of 0.4 mm. The coal was concentrated by flotation using 0.3 kilos cresol and 0.23 kilos kerosene oil per ton of coal, in which operation the ash content was reduced from 15% to 5%.

The concentrates removed had a water-solid ratio of 1.33 : 1.

The concentrates with their associated water were transferred to a vessel in which they were agitated as in Example I, and during the agitation the coal-tar product known as anthracene oil was added, the quantity of oil amounting to 3% of the weight of the dry concentrates. This operation was carried out at room temperature. An intense flocculation was produced, and when some of the wet flocculated coal was placed on a screen having 24 apertures per lineal centimeter, clear water ran through, and the greater part of the contained water drained away.

When the wet flocculated coal was placed in a mould having slits for egress of water and subjected to a pressure of 80 kilos per square cm., some further water exuded and a cake was formed which contained 12% water.

A pressure of 160 kilos per square cm. produced a cake containing 9% of water. In either case the cake crumbled easily in the fingers.

The cake was crumbled, packed into a silica pot, and heated for two hours at a

temperature rising gradually to 1040° C. Excellent coke suitable for metallurgical use was produced; it sustained a pressure of 160 kilograms per sq. cm. without crushing.

It is possible to effect not only the flocculation of the coal particles and the removal of the water therefrom, but also, in the same operation, it is possible to effect the separation of the gangue and other ash-forming materials from the coal particles.

Thus, according to this form of the invention, the finely divided coal particles, mixed with gangue or other ash-forming materials, are suspended in sufficient water to make a mobile pulp. This pulp is then subjected to agitation (preferably with aeration) with a flocculating agent of the kind hereinbefore described in quantity insufficient to form an amalgam in which the interstitial spaces between the particles would be filled with the agent but sufficient to coat the coal particles and flocculate them in water, the gangue particles not being so coated or flocculated, the gangue, with the water, being separated from the coal by draining or filtration, with or without pressure, but without the production of briquettes.

#### Example III

Waste coal or duff ground to pass a screen with 0.4 mm. aperture from the Powell Duffryn Mine in South Wales and containing 23.04% of ash was made up into a mobile pulp with an equal weight of water, and the pulp was agitated with the addition of 4.75% of by-product coke-oven coal-tar measured on the weight of the crude coal so as to produce flocculation. The wet flocculated coal was then transferred to a press and subjected to a pressure of 310 kilos per square cm. thereby extruding the water which carried the great proportion of the gangue. The resulting cake contained only 13% of ash and 5.56% of moisture. This test was carried out at normal atmospheric temperature.

The cake was crumbled, packed into a silica pot, and heated for two hours at a temperature rising gradually to 1040° C. Excellent coke suitable for metallurgical use was produced; it sustained a pressure of 160 kilograms per sq. cm. without crushing.

Again the process of flocculating the coal particles may be carried out in such a way that the coal particles are coated and flocculated and separated in the form of a float supported by bubbles while the gangue remains in the water, thus obtaining a float relatively free from ash as compared with the raw coal.

#### Example IV

The same material as in Example III, viz., pulverized waste coal or duff from the Powell Duffryn Mine in South Wales ground to pass a screen with 0.4 mm. aperture was

mixed with its own weight of water to form a mobile pulp. There was added to this pulp the following reagents:—

4.7% by-product coke-oven coal-tar,  
5 0.075% cresol, 0.075% kerosene oil, (these percentages being measured on the weight of crude coal).

After agitation and aeration the flocculated coal separated as a float supported by bubbles, 0 and was removed and subjected to a pressure of 310 kilos per square cm. The resulting cake contained only 5.76% of ash and 3.87% of moisture.

The cake was crumbled, packed into a silica pot, and heated for two hours at a temperature rising gradually to 1040° C. Excellent coke suitable for metallurgical use was produced; it sustained a pressure of 160 kilograms per sq. cm. without crushing.

60 This test was carried out at normal temperature.

This application is a division of our pending application Serial Number 602,251, filed November 20th, 1922, upon which Patent No. 1,606,867 was issued November 16, 1926.

Having thus described certain embodiments of our invention, we claim:—

1. A process for producing coke which consists in agitating an aqueous pulp of finely divided coal with a flocculating agent having the characteristics of both a frothing agent and a coating oil, so that the coal is flocculated and coated with a water-repellant coating having so little adhesiveness as not to cause the coal to form into briquettes under water-expelling pressure, separating and draining the flocculated coal, and coking the drained coal.

2. A process for producing coke which consists in agitating an aqueous pulp of finely divided coal with a flocculating agent containing both a water-soluble frothing agent and a coating oil, so that the coal is flocculated and coated with a water-repellant coating having so little adhesiveness as not to cause the coal to form into briquettes under water-expelling pressure, separating and draining the flocculated coal, and coking the drained coal.

50 3. A process for producing coke which consists in agitating an aqueous pulp of finely divided coal with a few per cent. of a coal tar under such conditions that the coal is flocculated and coated with a water-repellant coating having so little adhesiveness as not to cause the coal to form into briquettes under water-expelling pressure, separating and draining the flocculated coal, and coking the drained coal.

60 4. A process for producing coke which consists in agitating an aqueous pulp of finely divided coal with about three per cent. of a flocculating agent, so that the coal is flocculated and coated with a water-repellant coating having so little adhesiveness as not

to cause the coal to form into briquettes under water-expelling pressure, separating and draining the flocculated coal and coking the drained coal.

5. A process for producing coke which 70 consists in agitating an aqueous pulp of finely divided coal with a flocculating agent, so that the coal is flocculated and coated with a water-repellant coating having so little adhesiveness as not to cause the coal to form into briquettes under water-expelling pressure, separating the flocculated coal, draining it under a pressure of the order of magnitude of 160 kilograms to the square centimeter, and coking the drained coal.

6. A process for producing coke which 75 consists in agitating an aqueous pulp of finely divided coal with a few per cent. of a coal tar, so that the coal is flocculated and coated with a water-repellant coating having so little adhesiveness as not to cause the coal to form into briquettes under water-expelling pressure, separating the flocculated coal, draining it under a pressure of the order of magnitude of 160 kilograms to the square 80 centimeter, and coking the drained coal.

7. A process for producing a low-ash coke which consists in agitating an aqueous pulp of finely divided coal with a flocculating agent, so that the coal is flocculated and coated with a water-repellant coating having so little adhesiveness as not to cause the coal to form into briquettes under water-expelling pressure, separating the flocculated coal and draining it under water-expelling pressure, whereby the coal is obtained relatively dry and of diminished ash content, and coking the drained coal.

8. A process for producing a low-ash coke which consists in agitating an aqueous pulp of finely divided carbonized coal with a few per cent. of a coal coating and flocculating coal tar product, so that the coal is flocculated and coated with a water-repellant coating having so little adhesiveness as not to cause the coal to form into briquettes under water-expelling pressure, separating the flocculated coal and draining it under water-expelling pressure, whereby the coal is obtained relatively dry and of diminished ash 105 content, and coking the drained coal.

9. A process for producing a low-ash coke which consists in agitating an aqueous pulp of finely divided coal with a few per cent. of a coal tar, so that the coal is flocculated and coated with a water-repellant coating having so little adhesiveness as not to cause the coal to form into briquettes under water-expelling pressure, separating the flocculated coal and draining it under water-expelling pressure, whereby the fuel is obtained relatively dry and of diminished ash content, and coking the drained coal.

10. A process for producing a low-ash coke which consists in subjecting finely divided

- coal to froth-flotation concentration with a frothing agent to produce a coal concentrate of diminished ash content, agitating a mobile pulp of the concentrate with a few per cent. of a flocculating agent so that the coal is flocculated and coated with a water-repellant coating having so little adhesiveness as not to cause the coal to form into briquettes under water-expelling pressure, separating and draining the flocculated coal, and coking the drained coal.
11. A process for producing a low-ash coke which consists in subjecting finely divided coal to froth-flotation concentration with a frothing agent including a water soluble element to produce a coal concentrate of diminished ash content, agitating a mobile pulp of the concentrate with a few per cent. of a flocculating agent so that the coal is flocculated and coated with a water-repellant coating having so little adhesiveness as not to cause the coal to form into briquettes under water-expelling pressure, separating and draining the flocculated coal, and coking the drained coal.
12. A process for producing a low-ash coke which consists in subjecting finely divided coal to froth-flotation concentration with a frothing agent containing a few per cent. of a coal tar to produce a coal concentrate of diminished ash content, agitating a mobile pulp of the concentrate with a few per cent. of a flocculating agent so that the coal is flocculated and coated with a water-repellant coating having so little adhesiveness as not to cause the coal to form into briquettes under water-expelling pressure, separating and draining the flocculated coal, and coking the drained coal.
13. A process for producing a low-ash coke which consists in subjecting finely divided coal to froth-flotation concentration with a frothing agent containing a few per cent. of a coal tar and an oily substance, to produce a coal concentrate of diminished ash content, agitating a mobile pulp of the concentrate with a few per cent. of a flocculating agent so that the coal is flocculated and coated with a water-repellant coating having so little adhesiveness as not to cause the coal to form into briquettes under water-expelling pressure, separating and draining the flocculated coal, and coking the drained coal.
14. A process for producing a low-ash coke which consists in subjecting finely divided coal to froth-flotation concentration with a frothing agent, so that the coal is flocculated with diminished ash content and coated with a water-repellant coating having so little adhesiveness as not to cause the coal to form into briquettes under water-expelling pressure, separating the flocculated coal and draining it under water-expelling pressure, and coking the drained coal.
15. A process for producing a low-ash coke which consists in subjecting finely divided coal to a froth-flotation concentration with a few per cent. of a coal coating and flocculating coal tar product, so that the coal is flocculated with diminished ash content and coated with a water-repellant coating having so little adhesiveness as not to cause the coal to form into briquettes under water-expelling pressure, separating the flocculated coal and draining it under water-expelling pressure, and coking the drained coal.
16. A process for producing a low-ash coke which consists in subjecting finely divided coal to froth-flotation concentration with a few per cent. of a coal tar so that the coal is flocculated with diminished ash content and coated with a water-repellant coating having so little adhesiveness as not to cause the coal to form into briquettes under water-expelling pressure, separating the flocculated coal and draining it under water-expelling pressure, and coking the drained coal.
17. A process for producing a low-ash coke which consists in subjecting coal to froth-flotation concentration with a frothing agent containing a few per cent. of a coal tar so that the coal is flocculated with diminished ash content and coated with a water-repellant coating having so little adhesiveness as not to cause the coal to form into briquettes under water-expelling pressure, separating the flocculated coal and draining it under a pressure of the order of magnitude of 160 kilograms to the square centimeter, and coking the drained coal.
18. A process for producing a low-ash coke which consists in subjecting coal to froth-flotation concentration with a frothing agent containing a few per cent. of a coal coating and flocculating coal tar product, so that the coal is flocculated with diminished ash content and coated with a water-repellant coating having so little adhesiveness as not to cause the coal to form into briquettes under water-expelling pressure, separating the flocculated coal and draining it under a pressure of the order of magnitude of 160 kilograms to the square centimeter, and coking the drained coal.
19. A process for producing coke which consists in agitating an aqueous pulp of powdered coal with a flocculating agent so that the coal is flocculated and coated with a water-repellant coating adapted to be partly volatilized in a subsequent coking operation and having so little adhesiveness as not to cause the coal to form into briquettes under water-expelling pressure, separating and draining the flocculated coal, and coking the drained coal.
20. A process for producing coke which consists in agitating an aqueous pulp of powdered coal with a flocculating agent so that the coal is flocculated and coated with a wa-

ter-repellant coating adapted to be partly volatilized in a subsequent coking operation and having so little adhesiveness as not to cause the coal to form into briquettes under 5 water-expelling pressure, separating and draining the flocculated coal, coking the drained coal, and recovering volatilized flocculating agent.

21. A process for producing coke which 10 consists in agitating an aqueous pulp of powdered coal with a coal tar so that the coal is flocculated and coated with a water-repellant coating adapted to be partly volatilized in a subsequent coking operation and having so 15 little adhesiveness as not to cause the coal to form into briquettes under water-expelling pressure, separating and draining the flocculated coal and coking the drained coal.

22. A process of producing coke which 20 consists in agitating an aqueous pulp of powdered coal with a few per cent. of a flocculating agent so that the coal is flocculated and coated with a water-repellant coating adapted to be partly volatilized in a subsequent 25 coking operation and having so little adhesiveness as not to cause the coal to form into briquettes under water-expelling pressure, separating and draining the flocculated coal, and coking the drained coal.

26. 23. A process for producing a low-ash coke which consists in subjecting an aqueous pulp of powdered coal to froth-flotation concentration to form a concentrate of diminished ash content, agitating a mobile pulp of the 35 concentrate with a flocculating agent so that the coal is flocculated and coated with a water-repellant coating adapted to be partly volatilized in a subsequent coking operation and having so little adhesiveness as not to 40 cause the coal to form into briquettes under water-expelling pressure, separating and draining the flocculated coal, and coking the drained coal.

In testimony whereof we affix our signatures.

WALTER BROADBRIDGE.

EDWIN EDSER.

WILLIAM WARWICK STENNING.